

Feb. 25, 1947.

L. G. SELMI ET AL

2,416,649

ALLOY STEEL

Filed March 4, 1942

3 Sheets-Sheet 1



FIG. 1

INVENTOR  
LUCIANO G. SELMI and  
CLARENCE L. ALTBURGER  
BY  
Fay Machine Co.  
Williams, Shilton and Baker  
ATTORNEYS

Feb. 25, 1947.

L. G. SELMI ET AL

2,416,649

ALLOY STEEL

Filed March 4, 1942

3 Sheets-Sheet 2



FIG.2

BY

INVENTOR  
LUCIANO G. SELMI and  
CLARENCE L. ALTENDORGER  
Fay, Macklin, Golub  
Williams, Shultz and Selin  
ATTORNEYS

Feb. 25, 1947.

L. G. SELMI ET AL

2,416,649

ALLOY STEEL

Filed March 4, 1942

3 Sheets-Sheet 3



FIG. 3.

INVENTORS.

By *Tay Macklin Golick*  
LUCIANO G. SELMI and  
CLARENCE L. ALLENBURGER  
*Williams, Shultz and Selmi*

ATTORNEYS.

## UNITED STATES PATENT OFFICE

2,416,649

## ALLOY STEEL

Luciano G. Selmi, Detroit, and Clarence L. Altenburger, Dearborn, Mich., assignors to Great Lakes Steel Corporation, Ecorse, Mich., a corporation of Delaware

Application March 4, 1942, Serial No. 433,404

4 Claims. (Cl. 148—31)

1

This invention relates, as indicated, to alloy steels but has reference more particularly to alloy steels of the so-called low alloy types, examples of which have been described by the present applicants in previously granted United States Patents Nos. 2,234,130, now Reissue No. 22,072, and 2,250,505.

The low alloy steels of the present invention is characterized by an inherent fine-grained structure, high tensile strength, outstanding welding qualities, long fatigue life, ductility for deep drawing, and extremely high impact properties at normal as well as at sub-zero temperatures. Basically it is a low alloy steel, attaining high qualities and in which valuable alloying elements, and particularly those of present strategic importance, such as silicon, chromium and zirconium, are held to a minimum.

Another desirable characteristic of this steel when carburized is that the structure has no massive cementite network, such as constitutes a weakness of the hypereutectoid case produced in the carburizing of other steels. Further, we have found that both nickel and silicon prevent high carbon concentration in the case even when fairly large content of chromium is present. Same is true in respect to the presence of molybdenum when used as in the above named patents and co-pending application, Serial No. 433,384.

The invention sought to be covered by this present application and as hereinafter claimed is a steel having balanced relationships of the constituents such that, within the limits of sectional thicknesses, and under treatment conditions herein given, results are accomplished which have not been possible in previous high tensile, low alloy steels.

Other objects will become apparent from the following description.

The steel in addition to iron, contains the fol-

2

lowing elements intended in practice to be within the ranges specified:

|                | Per cent |
|----------------|----------|
| Carbon         | .08-.30  |
| 5 Manganese    | .30-.75  |
| Silicon        | .60-.90  |
| Chromium       | .30-.75  |
| Zirconium      | .06-.20  |
| Sulphur        | .03-max. |
| 10 Phosphorous | .03-max. |

A preferred steel within the foregoing range is one having the following analysis:

|                | Per cent         |
|----------------|------------------|
| 15 Carbon      | .13              |
| Manganese      | .66              |
| Silicon        | .80              |
| Chromium       | .54              |
| Zirconium      | .06-.13 variable |
| Sulphur        | .025             |
| 20 Phosphorous | .020             |

This particular steel, when used in "as rolled," or normalized condition, or when stress relieved for high tensile steel fabrication, possesses a resistance to fatigue and notched bar values at the strength levels of 50,000 p. s. i. minimum yield strength and 70,000 p. s. i. minimum tensile strength common to low alloy high tensile steels, and greater than those heretofore available.

25 This particular steel is further characterized by: (a) high grain coarsening temperatures upon normalizing, and only slight change in physical properties consequent upon increases in normalizing temperatures; (b) comparative freedom from blue brittleness and hence freedom from strain aging even in the normalized or "as rolled" conditions, and (c) good notched bar impact strength at normal and sub-zero temperatures. Other noteworthy properties of this particular steel are its excellent weldability as

well as the ability to be cold formed into various difficult shapes.

The effects of various conditioning heat treatments after hot rolling bar of the analyses indicated to various physical properties appear in the drawings and tables herein given.

Fig. 1 is a chart showing physical properties at different drawing temperatures.

Fig. 2 is a chart showing effect of drawing on physical properties.

Fig. 3 is a micro-photograph showing grain structure and size of our steel when carburized.

The following Table I gives physical properties of our steel as rolled finishing at temperatures from 1600° F. to 1650° F. producing 7 to 8 McQuaid Ehn grain size, according to the following Table II and Fig. 3.

TABLE I

| C   | Mn  | P    | S    | Si  | Cr  | Zr  |
|-----|-----|------|------|-----|-----|-----|
| .13 | .67 | .020 | .020 | .84 | .50 | .11 |

3/8" round finishing rolling temperatures 1600° F. to 1650° F.

[As rolled grain size 7 to 8]

|              | Tensile | Yield point | Elongation |    |    | Red. A. |
|--------------|---------|-------------|------------|----|----|---------|
|              |         |             | 2"         | 4" | 8" |         |
| Longitudinal | 72,475  | 53,000      | 52         | 37 | 27 | 67.9    |
| Transverse   | 71,000  | 50,200      | 46         | 34 | 25 | 58.6    |

TABLE II  
Carbon analysis of carburized specimen at temperature shown

| Depth of cut, inches | 1620° F.       | 1700° F.       | 1750° F.       |
|----------------------|----------------|----------------|----------------|
| 0.0-0.005"           | Carbon %, 1.05 | Carbon %, 1.05 | Carbon %, 1.21 |
| 0.005-0.010"         | Carbon %, .90  | Carbon %, 1.00 | Carbon %, 1.07 |
| 0.010-0.015"         | Carbon %, .84  | Carbon %, .94  | Carbon %, 1.05 |
| 0.015-0.020"         | Carbon %, .77  | Carbon %, .92  | Carbon %, .99  |
| 0.020-0.025"         | Carbon %, .72  | Carbon %, .85  | Carbon %, .95  |
| 0.025-0.030"         | Carbon %, .65  | Carbon %, .81  | Carbon %, .91  |
| 0.030-0.040"         | Carbon %, .57  | Carbon %, .75  | Carbon %, .87  |
| Grain size           | 96             | 96             | 96             |

The analysis of this steel is as follows:

|            | Per cent |
|------------|----------|
| Carbon     | .12      |
| Manganese  | .66      |
| Phosphorus | .026     |
| Sulphur    | .025     |
| Silicon    | .85      |
| Chromium   | .54      |
| Zirconium  | .13      |

Carbon percentages in excess of eutectoid carbon may be accurately determined by analyzing lathe turnings taken at prescribed depths from the surface as shown in Table II. Carbon concentrations when using standard grades of carburizing compound in our steel is as indicated in the above table at varying carburizing temperatures. The time at temperatures given being eight hours and the furnace being cooled from the carburizing temperature.

The following Table III gives properties of a similar steel as rolled and normalized at the temperatures given, i. e. 1575° F. to 1850° F. and as listed, the yield point, tensile (or ultimate)

strength, elongation in 2, 4, 6, and 8 inches and reduction of area.

TABLE III

|    | Yield point | Tensile strength | Elongation |    |        |      | Red. A. |       |
|----|-------------|------------------|------------|----|--------|------|---------|-------|
|    |             |                  | 2"         | 4" | 6"     | 8"   |         |       |
| 10 | As rolled   | 54,500           | 73,500     | 42 | 30 1/2 | 29.7 | 25.5    | 74.4  |
|    | Normalized: |                  |            |    |        |      |         |       |
|    | 1575° F.    | 54,000           | 72,500     | 42 | 33     | 28.1 | 27      | 75.6  |
|    | 1600° F.    | 52,500           | 72,000     | 42 | 34     | 28.8 | 28.7    | 75.9  |
|    | 1625° F.    | 52,500           | 72,000     | 42 | 33     | 30.7 | 28.1    | 75.5  |
|    | 1700° F.    | 52,000           | 71,500     | 42 | 33     | 28.8 | 26      | 75.1  |
|    | 1750° F.    | 50,500           | 71,000     | 42 | 32     | 29.5 | 27.4    | 76    |
|    | 1800° F.    | 50,000           | 71,000     | 42 | 31.6   | 28.6 | 27.7    | 74.90 |
|    | 1850° F.    | 47,000           | 70,500     | 42 | 30     | 26   | 24.5    | 74.7  |

Table IV shows Charpy key hole impact strength at 75° F., on the longitudinal and transverse, at 30° F., at 0° F., minus 50° F., and at minus 100° F.

TABLE IV

|    | Karpay key hole test |                  |                    |                    |                     |
|----|----------------------|------------------|--------------------|--------------------|---------------------|
|    | 75° F.               | 32° F.           | 0° F.              | Minus 50° F.       | Minus 100° F.       |
| 25 | Y. P.<br>67.7        | Y. P.<br>64      | Y. P.<br>60        | Y. P.<br>53        | Y. P.<br>41.5       |
|    | Transverse<br>48.5   | Transverse<br>45 | Transverse<br>41.5 | Transverse<br>35.5 | Transverse<br>24.00 |

End quenched Rockwell C hardness of our steels of similar analyses are given in the following Tables V and VI.

TABLE V

|    | End quench analysis                 | Hardness Rockwell C.<br>Rockwell C.                                                                                   |
|----|-------------------------------------|-----------------------------------------------------------------------------------------------------------------------|
| 40 | C<br>Mn<br>P<br>S<br>Si<br>Cr<br>Zr | 14<br>74<br>.012<br>.027<br>.85<br>.70<br>.17                                                                         |
| 45 |                                     | 1 1/2".....40<br>2 1/2".....35<br>3 1/2".....30<br>4".....24<br>5".....14<br>5 1/2".....8<br>6".....9<br>1 1/4".....6 |

TABLE VI

|    | End quench analysis                 | Hardness Rockwell C.<br>Rockwell C.                                                                                                 |
|----|-------------------------------------|-------------------------------------------------------------------------------------------------------------------------------------|
| 50 |                                     | 1 1/2".....43<br>2 1/2".....40<br>3 1/2".....34<br>4".....30<br>5".....20<br>5 1/2".....18<br>6".....12<br>7".....8<br>1 1/4".....7 |
| 55 | C<br>Mn<br>P<br>S<br>Si<br>Cr<br>Zr | .16<br>.64<br>.012<br>.025<br>.76<br>.67<br>.15                                                                                     |

It should be noted that heating above the AC<sub>3</sub> point brings the physicals to almost the same value.

The physical properties can be raised considerably by cold drawing. Cold drawing lowers the proportional limit but this can be raised considerably by a short draw, as shown in the accompanying drawing, Fig. 2, in which the effect of a one hour draw on the physical properties of cold drawn bar on a steel of approximately the preferred analysis after 19.5% cold reduction is graphically illustrated.

The weldability of this alloy steel is exceptionally good.

For one bead weld the Rockwell B hardness when the parent metal is 85 the Rockwell B

hardness in the heat affected zone will not exceed 92 Rockwell B.

Hardness lower than 92 Rockwell B is attained in the heat affected zone in multiple bead welds.

TABLE VII  
Plain end quench bar test 1" diameter x 3" long  
Rockwell C hardness

| Distance 16th"           | 15    | 20    | 30    |       |
|--------------------------|-------|-------|-------|-------|
| 1                        | 40    | 43    | 44    | 44    |
| 2                        | 35    | 40    | 42    | 44    |
| 3                        | 30    | 34    | 37    | 40    |
| 4                        | 24    | 30    | 32    | 35    |
| 5                        |       |       |       | 47    |
| 6                        | 19    | 22    | 25    | 26    |
| 7                        |       |       |       | 35    |
| 8                        | 14    | 18    | 20    | 21    |
| 10                       |       |       |       | 30    |
| 12                       | 8     | 12    | 15    | 14    |
| 14                       |       |       |       | 24    |
| 16                       | 8     | 8     | 8     | 10    |
| 20                       | 6     | 7     | 8     | 8     |
| 24                       | 6     | 6     | 8     | 8     |
| 28                       | 5     | 5     | 7     | 7     |
| 32                       | 5     | 5     | 6     | 8     |
| Grain size               | Fine  | Fine  | Fine  | Fine  |
| Quench. temp., degrees F | 1,630 | 1,630 | 1,630 | 1,575 |
| C                        | .14   | .16   | .18   | .20   |
| Mn                       | .74   | .64   | .70   | .72   |
| P                        | .012  | .012  | .010  | .012  |
| S                        | .027  | .025  | .025  | .023  |
| Si                       | 1.05  | .76   | .71   | .84   |
| Cr                       | .70   | .67   | .66   | .68   |
| Zr                       | .17   | .15   | .17   | .23   |

Steels made in accordance with the present invention are especially valuable for use in the manufacture of most armament appliances, either "as rolled" or heat treated. Typical applications are for tanks, gun carriages, transport trailers, frames of Jeep buggies, tractors, road scrapers, busses and railroad cars, airplane frames, etc.

Our steel of such composition as given and described will under carburizing treatment with solid, liquid or gaseous cementing medium produce an hypereutectoid case practically free of cementite network as shown in microphotograph, Fig. 3. Such hypereutectoid case free of cementite network is much stronger and more desirable in hard wearing surface such as required in gears, pinions, etc., which will spall off if the hypereutectoid case is made up of cementite network.

Having thus described our invention, the nature and scope thereof are defined in the appended claims, it being understood that the particular relationships and ranges specified may be subject to slight or reasonable variation without departing from the spirit of our invention.

We claim:

1. A case carburized steel article formed from chromium carburizing steel containing as essential alloying elements, 0.1 to about 0.3 per cent of carbon, from about 0.5 to about 0.75 per cent of chromium, about 0.6 to about 0.9 per cent of

silicon, .06 to .20 per cent of zirconium, and substantially no nickel, and the remainder iron together with impurities and elements in amounts which do not adversely affect the carburizing characteristics of the steel, and characterized by the carburized and hardened case being resistant to spalling and low in or substantially free from massive carbides.

2. A chromium-containing carburized steel article containing as essential alloying elements about 0.5 to about 0.75 per cent of chromium, about 0.6 to about 0.9 per cent of silicon, .06 to .20 per cent of zirconium, carbon from 0.1 to about 0.3 per cent and in an amount such that the steel is hardenable by heat treatment, and the remainder iron together with impurities and elements in amounts which do not adversely affect the carburizing and heat treating characteristics of the steel, and characterized by a carburized case resistant to spalling and low in or substantially free from massive carbides, and high tensile strength in the core as the result of heat treatment.

3. A nickel-free carburized steel article containing as essential alloying elements from about 0.1 to about 0.3 per cent of carbon, about 0.5 to about 0.75 per cent of chromium, about 0.6 to about 0.9 per cent of silicon, .06 to .20 per cent of zirconium, and substantially no nickel, and the remainder iron together with impurities and elements in amounts which do not adversely affect the carburizing characteristics of the steel, and characterized by a carburized case resistant to spalling and low in or substantially free from massive carbides.

4. A case carburized steel article formed from chromium carburizing steel containing as essential alloying elements about 0.1 to about 0.3 per cent of carbon, about 0.5 to 0.75 per cent of chromium, about 0.6 to about 0.9 per cent of silicon, .06 to .20 per cent of zirconium, and the remainder iron together with impurities and elements in amounts which do not adversely affect the carburizing characteristics of the steel, and characterized by the carburized and hardened case being resistant to spalling and low in or substantially free from massive carbides.

LUCIANO G. SELMI.

CLARENCE L. ALTBURGER.

#### REFERENCES CITED

The following references are of record in the file of this patent:

#### UNITED STATES PATENTS

| Number    | Name   | Date          |
|-----------|--------|---------------|
| 2,114,802 | Kinzel | Apr. 19, 1938 |
| 2,250,505 | Selmi  | July 29, 1941 |
| 2,152,434 | Kinzel | Mar. 28, 1939 |